

April 27, 1937.

J. G. MALONE

2,078,917

METHOD OF ATTACHING RUBBER TO METAL AND ARTICLES PRODUCED THEREBY

Filed Aug. 24, 1934

*Fig. 1.*



*Fig. 2.*



INVENTOR  
JOHN GILBERT MALONE  
BY  
Walter L. Pipes  
ATTORNEY

## UNITED STATES PATENT OFFICE

2,078,917

METHOD OF ATTACHING RUBBER TO  
METAL AND ARTICLES PRODUCED  
THEREBY

John Gilbert Malone, Detroit, Mich., assignor, by  
mesne assignments, to United States Rubber  
Company, New York, N. Y., a corporation of  
New Jersey

Application August 24, 1934, Serial No. 741,200

7 Claims.

(CL. 18—59)

This invention relates to attaching rubber to metal and more particularly to ferrous metal.

In the present commercial practice of preparing ferrous metal bases for adhesion with rubber, a plating of brass is deposited electrolytically on the base from a cyanide solution of copper and zinc, using a brass anode. In order to obtain proper adhesion of the rubber to such a plating, it is necessary for the copper and zinc to be deposited in definite proportions, about a 75% copper and 25% zinc combination producing optimum results. The proportions of copper and zinc, however, can only be controlled in an electro plating operation when the metal surface to be treated is comparatively uniform in plane and is located in the bath at a definite relative position to the anode. Where the article to be rubber coated is uneven and irregular in shape, the composition of the copper and zinc in a deposit on the base is not maintained uniform, nor for that matter, is the thickness of the deposit. In plating an uneven surface more metal deposits on the elevated portions and on the edges than in the depressions. This variation of thickness caused by directional effect may be as much as 1 to 10 for different parts of the surface. Also, a greater percentage of copper is deposited in the depressions or hollow portions and a higher percentage of zinc is deposited along the projections or edges of the article. The importance of obtaining a uniformly proportionate deposit of the copper and zinc is exemplified when it is considered that on the basis of 100% adhesion quality for a 75% copper and 25% zinc combination, a 100% copper plating produces an adhesion quality of about 50%, and where the copper content drops to about 60% with about 40% zinc content, the adhesion quality of the rubber to the copper-zinc plating is practically nil. It has long since been suggested that rubber be adhered to metal by first "dip-coating" the metal with copper from a copper sulphate solution, but as seen in the figures above, such a coating on the base metal provides an adhesion quality only half that obtainable with a 75% copper and 25% zinc coating.

According to the present invention, high quality adhesion of rubber to metal may be obtained by means of an alloy surface which may be deposited by a so-called "dip-coating" method. By "dip-coating" a metal base is meant the treatment of the base with a solution of the metals desired to be plated by a dipping, spraying, spreading or other operation and allowing the plating operation to proceed merely by contact

of the liquid with the base without the aid of an external electric current as in an electro plating operation. The metal surface to which the rubber may be adhered according to the present invention is a bronze surface, that is, an alloy comprising a major proportion of copper and a minor proportion of tin, with or without small amounts of other metals, as is well known in the art.

In the accompanying drawing: 10  
Fig. 1 is a perspective view showing a sheet of rubber secured to a metallic plate in accordance with the invention; and

Fig. 2 is a cross sectional view on the lines 2—2 of Fig. 1. 15

Referring more particularly to the drawing, 10 illustrates a metal plate with a bronze coating 11 to which is vulcanized the rubber composition 12. 15

In carrying out the present invention, the 20 metal, commonly a ferrous metal, to which rubber is to be secured, is provided with a bronze surface preferably by a "dip-coating" method, although an electro plating method or a melting of the alloy directly on the surface of the base 25

may be employed. 20  
The following example of coating a steel base with rubber by first "dip-coating" the base with bronze is included merely as an illustration of the present invention and is not to be considered as limiting the same. 30  
The steel base was one designated in the trade as a 10—10 carbon steel, hot rolled. It contains about .02% sulphur, .007% phosphorus, .37% manganese, and .06% carbon. The micro structure is considered ferrite 35 with minute pearlite areas with no evidence of deformation due to cold working. This is merely illustrative of the type of material which in large quantities is coated with a rubber composition in commercial practice. The constituents of the 40 plating solution were Sn, which may be added as  $\text{SnCl}_2$ ; Cu, which may be added as  $\text{CuSO}_4$ ; and oxalate, which may be added as potassium, sodium or ammonium oxalate, or as oxalic acid which is preferably almost completely neutralized 45 by hydroxide. An example of a satisfactory solution contains 2 to 3 ounces of oxalate per gallon prepared by neutralizing all but about .5 oz. per gallon of the oxalic acid with potassium, sodium, or ammonium hydroxide to a phenolphthalein 50 end point; .05 to .15 oz. per gallon of Sn as  $\text{SnCl}_2 \cdot 2\text{H}_2\text{O}$ ; .002 oz. per gallon of copper as disodium (or ammonium) diaquo dioxalate cuprate prepared by adding copper sulphate to a hot solution of sodium oxalate, as for example, 55

by adding a saturated copper sulphate solution to a solution containing about 5 oz. of sodium oxalate per gallon until turbidity appears. The disodium (or ammonium) diaquo dioxalate may be prepared as described by Fink and Wong Trans. Electrochem. Soc., Vol. 63, pages 67-68, (1933). The coating solution should at all times be kept acid and it is preferable to apply the solution at a temperature between 50 and 60° C. 5

10 A five minute treatment with the solution at such temperature is satisfactory but a longer treatment is not detrimental. The surface may be coated by dipping into the solution or by spraying the solution on to the surface, using a compressed air operated spray jet. The metal and the spray gun, however, should be free from oil 15 and grease or a uniform plating cannot be attained. A so-called rubber adhesion stock containing a vulcanizing agent was brought into 20 contact with the dried bronze-coated steel base and vulcanized to the bronze coating by a heating operation as in present practice. An adhesion stock which is satisfactory on a bronzed surface is set forth below, but many other different adhesion stocks may be used and these 25 are well known in the art of adhering rubber to metal surfaces:

|                           |     |
|---------------------------|-----|
| Rubber                    | 38  |
| Whiting                   | 44  |
| 30 Softener               | 9.6 |
| Carbon black              | 4   |
| Sulphur                   | 1.1 |
| Zinc oxide                | 2.3 |
| Diphenylguanidine         | .5  |
| 35 Semi-rapid accelerator | .3  |
| Antioxidant               | .2  |

The above composition may be vulcanized to the metal by heating for one-half hour at 148° C. 40 A bronze coating plated on a metal by a dip-coating method, unlike brass coated on a metal by an electroplating method, is of uniform thickness even over irregular portions of the article, and is of uniform composition at the same depth of the coating throughout the article. 45 However, a dip-coating of bronze unlike the usual electroplated coatings gives a great variation in composition in the various layers of the coating itself, and a bulk analysis of the coatings is not a fair guide in determining the analysis of the coating for the best adhesion to a particular stock. The bulk analysis of satisfactory coatings shows generally about 20% tin and over, but the color of the outer layers of the plating is a 50 much better guide than bulk analysis and should be gold when deposited from an oxalato-copper-tin solution. The proportion of copper to tin increases as the deposition continues and is materially greater on the outer surface of the coatings than adjacent the base. Analysis of the best coatings for adhesion show as a rule less than 15% tin in the outer coating layers, but with some stocks satisfactory adhesion may be obtained on a surface having as high a tin content 55 as 30%, which is considerably more than the usual run of commercial bronzes. It is considered that this variation in the proportion of the different ingredients of the alloy between the outer surface of the coating and the surface adjacent the base may be a considerable factor in the production of successful coatings by the present invention.

The example above shows a dip-coating of bronze on ferrous metal for adhesion of rubber 75 to ferrous metal, but the bronze may be coated

on any metal base to which it is desired to adhere the rubber stock. As above stated, the bronze may, if desired, be coated on the metal stock by melting the same on to a clean surface of the stock, or by an electroplating, as well as by a dip-coating process, as above described. If it is desired to adhere a rubber composition to a bronze base and the base is of a proper composition for securing the desired rubber composition, no auxiliary coating of course need be applied and the stock may be secured directly on to a cleaned surface of the base. If the bronze is too high in tin, it may be dip-coated with an axalato-copper-tin solution as above described. If, however, the bronze is of too high a 15 copper content, or if, for example, it is desired to secure rubber directly to a copper surface, then it is necessary to first plate the high-copper bronze or the copper base with a metal, such as tin, to which both the base and the desired dip-coated bronze surface will adhere. For example, in dip-coating a copper surface, the cleaned copper surface may be coated with  $\text{SnCl}_2$  and water in the form of a paste which is then rubbed well with a wire brush to produce a tinned surface to which after washing the bronze may be applied by the dip-coating method as above. The same method is applicable in the case of a high-copper bronze where it is desired to plate a 20 bronze coating of lower copper content for the 25 desired adhesion.

By dip-coating the base with an acid aqueous oxalate solution containing copper and tin, coatings having less tendency to "stain spotting" than coatings from alkaline cyanide solutions as 35 in brass electro-plating are obtained, since it is known that alkaline compounds are more likely to cause this spotting out than acid substances. This spotting out is believed to deleteriously affect the adhesion of the rubber, and experiments 40 have shown that a small amount of residual oxalic acid on the metal coating does not impair adhesion of the rubber composition while small amounts of residual cyanide do.

The bronze surface of the metallic base may 45 contain various proportions of copper and tin for different adhesion stocks, and may be coated or plated on the base by a variety of methods, as above described. The various rubber adhesion stocks may be vulcanized on to the metal surface 50 at various temperatures and for different periods of time depending on the composition of the same as is well known in the art. Various modifications of the invention will occur to those skilled in the art and it is not intended to limit the 55 invention other than as set forth in the appended claims.

Having thus described my invention, what I claim and desire to protect by Letters Patent is:

1. A new article of manufacture comprising a 60 ferrous base, a bronze coating comprising a major proportion of copper and a minor proportion of tin on said base, the proportion of copper to tin in said bronze being materially greater on the outer surface of said coating than adjacent the 65 said base, the tin content of said outer surface being up to 15 percent and a rubber layer vulcanized on said coating.

2. A new article of manufacture comprising a 70 metallic base, a bronze coating comprising a major proportion of copper and a minor proportion of tin on said base, the proportion of copper to tin in said bronze being materially greater on the outer surface of said coating than adjacent the 75 said base, analysis of the outer surface of the

coating showing at the most 15% tin and bulk analysis of the entire thickness of coating showing at least 20% tin, and a rubber layer vulcanized on said coating.

5 3. A new article of manufacture comprising a ferrous base, a bronze coating comprising a major proportion of copper and a minor proportion of tin on said base, the proportion of copper to tin in said bronze being materially greater on the 10 outer surface of said coating than adjacent the said base, analysis of the outer surface of the coating showing at the most 15% tin and bulk analysis of the entire thickness of coating showing at least 20% tin, and a rubber layer vulcanized 15 on said coating.

4. The method of attaching rubber to metal which comprises dip-coating a bronze containing up to 15 percent tin in the outer layers upon the 20 metal from a solution containing copper and tin, bringing rubber containing a vulcanizing agent into engagement with the coated surface, and vulcanizing the rubber onto said surface.

5. The method of attaching rubber to ferrous metal which comprises dip-coating a bronze containing up to 15 percent tin in the outer layers 25

upon the ferrous metal from an aqueous solution containing copper and tin, bringing rubber containing a vulcanizing agent into engagement with the coated surface, and vulcanizing the rubber onto said surface.

6. The method of attaching rubber to metal which comprises dip-coating a bronze containing up to 15 percent tin in the outer layers and with a bulk analysis of the entire thickness of the coating showing at least 20 percent tin upon the metal 10 from an aqueous solution containing copper and tin, bringing rubber containing a vulcanizing agent into engagement with the coated surface, and vulcanizing the rubber onto said surface.

7. The method of attaching rubber to ferrous 15 metal which comprises dip-coating a bronze containing up to 15 percent tin in the outer layers and with a bulk analysis of the entire thickness of the coating showing at least 20 percent tin upon the metal from an aqueous solution containing copper and tin, bringing rubber containing a vulcanizing agent into engagement with the 20 coated surface, and vulcanizing the rubber onto said surface.

JOHN GILBERT MALONE. 25